

Nov. 2, 1937.

H. E. WALTERS

2,097,709

METHOD OF MAKING ROLLS

Filed Sept. 30, 1935

2 Sheets-Sheet 1

Fig. 1.



WITNESSES

A. B. Wallace.  
A. H. Dedham

INVENTOR.

Harry E. Walters  
BY Brown, Critchlow & Flick

ATTORNEYS.

Nov. 2, 1937.

H. E. WALTERS

2,097,709

METHOD OF MAKING ROLLS

Filed Sept. 30, 1935

2 Sheets-Sheet 2

Fig. 2.



Fig. 4.

Fig. 3.

Fig. 5.



WITNESSES

A. Wallace.  
A. Oldham

INVENTOR.

Harry E. Walters  
BY Brown, Critchlow & Flick

his ATTORNEYS.

## UNITED STATES PATENT OFFICE

2,097,709

## METHOD OF MAKING ROLLS

Harry E. Walters, Pittsburgh, Pa., assignor to  
United Engineering & Foundry Company,  
Pittsburgh, Pa., a corporation of Pennsylvania

Application September 30, 1935, Serial No. 42,800

7 Claims. (Cl. 22—205)

This invention relates to an improved process for making cast metal rolls, as used in metal rolling mills.

It has long been desirable to produce a cast metal roll, for example, to be employed in metal strip rolling operations, which roll is very resistant to scarring as caused by the ends of the strip passing through the rolls or by other means. Moreover, in recent years the severe drafts and speedier production methods as well as the work with wider and alloyed strip have made the advantages of a hard-surfaced roll particularly attractive. It is the usual practice to employ hard-surfaced rolls in the strip finishing mills, but in addition the use of hard-surfaced rolls in the regular mills is also highly beneficial.

Prior to my invention hard-surfaced rolls have been made by casting highly alloyed iron in a mold having a chilling surface adjacent the enlarged central portion of the roll. It has been found that this method produces a satisfactory surface on the enlarged central or working portion of the roll, but that the bearing necks and wabbler portions of the rolls are also of the same hard high alloy material. This means that in order to finish the roll after casting, the entire roll surface, including the central portion and the reduced neck portions, must be ground down rather than turned down by edge tools in a roll lathe.

Grinding the roll surfaces, and particularly the bearing necks and wabbler portions, has added greatly to the cost of manufacture since grinding is necessarily slow and expensive where the fillets, shoulders and other irregularly shaped bearing necks or other roll portions must be brought to the proper dimension and finish. The grinding of the truly cylindrical central portion of the roll is not difficult, nor does it noticeably add to the cost of roll manufacture over the cost of edge tool machining. Likewise, the enlarged central portion of the roll can usually be cast more closely to its finished size in that it contacts directly with an iron or other chill which is not the case with respect to the necks and wabbler.

I have also found that by former practices as above described sacrifice of strength and toughness in the roll must be made to obtain the hard roll surface. The alloy metal is more brittle and less adapted to withstand wear and shock than is a softer but tougher metal.

It has likewise been proposed to form composite rolls of different metals by casting. Difficulties of separation after freezing and lack of segregation have been experienced, however.

It is accordingly the object of my invention to avoid and overcome the foregoing and other difficulties of known rolls and methods of making them, and I provide a composite metal roll having an extremely hard working surface on its en-

larged portion but with a core of relatively soft tough metal extending through the central portion and forming the necks and wabbler and bonded by casting with the hard working surface.

Another object of my invention is to provide a method of casting composite rolls from different metals so that the roll will be tough and long-wearing in service and have a hard chilled working surface.

Another object of the invention is to provide a method of making rolls which are very hard on their working surface but in which the bearing necks and wabbler portions are relatively soft and can be edge-tool machined to size after casting.

The foregoing and other objects of the invention are achieved by casting a composite roll with reduced neck portions by bottom-pouring the central portion and lower neck with a hard alloy metal. The metal is surface-chilled at the central portion of the roll, and while all but the chilled shell of the metal is still molten bottom-pouring is continued, but with a softer metal. This displaces the molten alloy metal completely from the inside of the chilled shell of alloy metal and the casting of the roll is completed by top-pouring the upper bearing neck with the soft metal. The resulting composite roll includes a large central portion having a relatively soft metal core extending through the central portion and forming reduced bearing necks with a chilled relatively hard alloy metal shell forming the surface of the central roll portion and bonded to the core by casting.

In the drawings, Fig. 1 is a vertical cross-sectional view of typical apparatus which may be employed to practice the invention; Fig. 2 is a side elevation of a roll embodying the features of and constructed in accordance with the method of my invention; Fig. 3 is a transverse cross-sectional view taken on line III—III of Fig. 2; Fig. 4 is a transverse cross-sectional view taken on line IV—IV of Fig. 2; and Fig. 5 is a transverse cross-sectional view taken on line V—V of Fig. 2.

The principles of my invention are applicable to the manufacture of cast metal rolls of various shapes and sizes and adapted for any desired use. However, the invention is particularly concerned with the production of cast metal rolls for use in rolling metal strip and the like, and accordingly the invention has been illustrated and will be described as dealing with the manufacture of a relatively large and heavy strip mill roll.

Referring to Fig. 1 of the drawings, the numeral 10 indicates generally a mold formed of cylindrical flasks 11, 12, and 13 and a cylindrical chill 14 all secured together in vertical alignment by clamps 18. The cylindrical flasks 11, 12, and 13 are filled with molding sand or other refractory material 20 and 21 and are shaped with a pat-

tern (not shown) in the usual manner to define the molding cavity marked 23. The mold is adapted to be bottom-poured and to this end a vertically extending gate 26, lined with refractory 27, is provided. The gate 26 is formed with a basin 28 at its upper end and the gate extends into the mold cavity 23 at its bottom and in a direction substantially tangential to the mold cavity so that metal poured in the mold swirls in a circle about the cavity. Tangential pouring itself is old and well known and will not be described in greater detail.

An important feature of the invention is the provision in the mold just described of an overflow or drainage spout 31 lined with refractory 32 and provided with a closure plug 33. The overflow spout 31 may extend over a ladle 35 to deposit any overflow metal in the ladle. The overflow spout 31 is positioned in the mold slightly above the enlarged central portion of the roll which is defined by the chill 14.

In the practice of my invention the mold is bottom-poured through the gate 26 ordinarily with a relatively hard high alloy metal such as, for example, one of a composition comprising 2.84% carbon, .28% silicon, .07% sulfur, .14% manganese, .41% chromium, .30% molybdenum, .38% phosphorus, 4.05% nickel, and the remainder iron. The bottom-pouring of the mold is continued until the metal overflows through the spout 31 into the ladle 35. The closure plug 33 of the spout 31 is in the open position at this time. Bottom-pouring is then discontinued and the relatively hard metal is allowed to set for a time sufficient to cause the surface chilling of the metal at the enlarged central portion of the roll by the cylindrical chill 14. The action of the chill is such that the metal immediately adjacent or close to the surface of the chill, such as identified by the numeral 40 in Fig. 1, is frozen without precipitation of any carbon in the form of graphite. The carbon is retained in combined form in the metal and affords a very hard chilled surface on the finished roll. The metal marked 41 in Fig. 1 immediately below the chilled roll metal is also frozen, but since the chilling action is not so rapid at some distance from the chill surface, carbon is precipitated out of solution or from its combined form and appears as graphite 48 in the metal. Actually instead of two distinct layers of metal 40 and 41 as shown in the drawings, the change from the chill surface 14 inwardly of the roll is a gradual one in which more and more carbon is in the free or uncombined state.

After the metal layers 40 and 41 have solidified against the cylindrical chill 14 and while the remainder of the hard alloy metal is in a molten state the bottom-pouring of the mold is renewed. However, the mold is now poured with a relatively soft metal as, for example, ordinary gray cast iron, a typical composition being: carbon 3.3%, silicon .9%, phosphorus .35%, sulfur .1%, manganese .3%, and the remainder largely iron. The addition of the hot soft metal at the bottom of the mold together with the swirling action imparted to the metal by the tangential bottom feed causes the hard alloy metal still in the molten state to be carried up to and out of the overflow spout 31 into the ladle 35. The bottom-pouring of the softer metal is continued until all of the hard metal alloy has been forced by displacement out of the mold with the softer metal taking its place. The rotary movement of the metal is advantageous as a better washing and displacing action is obtained with a superior bond ultimately result-

ing between the softer core metal and the harder chilled surface metal.

The plug 33 in the overflow spout 31 is now closed and with the metal in the mold up to about the dotted line 45 the remainder of the mold is top-poured with the relatively soft core or neck-forming metal. The entire cast roll is then allowed to solidify in the usual manner and is ready for machining. The machining operations are quite simplified since the bearing neck and wabbler portions of the roll are of relatively soft gray cast iron and these portions can be tool-machined in an ordinary roll lathe. The enlarged central portion of the roll has an extremely hard surface which must be ground to size, but this can be readily accomplished by grinding since the surface is cylindrical.

The advantages of the process just described as well as the superior product resulting will be evident from a consideration of Figs. 2 to 5. The reduced bearing necks of the roll are shown in Figs. 3 and 5 and it will be seen that the sections as cast are relatively free from a chilling action and that the composition of the metal is substantially uniform from the surface of the roll inwardly to the axis. Due to the slow cooling of these portions of the roll, graphite, as represented by the marks 48, is precipitated quite uniformly throughout the bearing necks.

Sharply distinguishing from the bearing neck 30 sections of Figs. 3 and 5, is the central roll section, shown in Fig. 4, in which the numeral 40 indicates the outer layer or shell of hard alloy metal which has been highly chilled by direct contact with the cylindrical chill 14 so that substantially all of the carbon in the metal is retained in the combined state. The metal layer or shell 41 positioned internally of the layer 40 is also of the hard metal alloy, but some graphite has been precipitated into the metal as this portion of the roll has cooled somewhat slowly. The core of the roll which is of relatively soft metal is identified by the numeral 49 and graphite 48 is precipitated quite uniformly through the metal due to the slow cooling of this portion of the roll.

The bond between the hard alloy metal shell and the relatively soft core and neck metal is very satisfactory due to the thorough washing out of the original molten hard metal and the integral casting and cooling of the composite parts. The fact that the hard metal of the shell has a gradually changing combined carbon content further effects a substantial bonding action since there is not so sharp a line of demarcation between the metals, particularly with respect to the combined carbon content. Moreover, as shown in the drawings, there is a mechanical interlocking of the hard metal and softer metal as occasioned by the slightly uneven freezing of the hard metal and the uneven displacement of the original molten hard metal by the softer molten metal.

A modification or alternative of the method just described comprises first bottom-pouring with the hard alloy metal and chilling and then continuing the bottom-pouring with a softer tougher metal, all as described heretofore. However, the bottom-pouring with the softer metal is stopped after the molten hard alloy metal is displaced from the lower bearing neck. The spout 31 is then plugged and the upper bearing neck is poured as before with the softer metal. This process produces a roll having a large central portion of hard alloy metal and reduced necks of tougher but machinable metal.

The location of the overflow spout 31 is particularly important since to place it at the top of the mold would seriously prejudice, if not prevent, the operation of my improved process as diss-  
 5 placing and washing out the molten harder metal with a softer core metal would result in freezing of portions of the hard metal along the upper bearing neck and wabbler portions of the roll: By placing the overflow spout immediately above  
 10 the enlarged central portion of the roll the molten harder metal can be readily removed from the mold to obtain the effective result above described.

By way of illustrating the advantages of my invention, a typical scleroscope hardness reading on a known type of solid alloy roll cast in a mold having a chill only at the enlarged central portion of the roll showed a reading of 80 to 85 at the chilled central portion of the roll. The reading at the surface of the bearing necks cast against a refractory surface was 70 to 75. This reading in itself is a clear indication that grinding must be resorted to for finishing the roll.

As directly distinguished from the extreme hardness of both the central and neck portions of the roll just described is the composition of a roll constructed in accordance with the principles of the present invention. More particularly, a scleroscope hardness test made of a roll cast as heretofore described shows that the wabbler and bearing neck portions of the roll are substantially soft, namely, about 40 to 50. This is the standard scleroscope reading of ordinary gray iron. Metal of this degree of hardness can readily be tooled with usual machine tools in a lathe so that the machining of the roll necks is readily accomplished. The surface of the central portion of my improved roll is, however, extremely hard with, for example, the particular alloy metal recited, and the scleroscope reading is about 80 to 85. This surface is substantially cylindrical and can be cast close to finished size against a chill so that the central roll portion can be readily ground to size as will be understood.

I have found that there is very little change in the percentage of free carbon in a radially outward direction from the axis of the roll except in the chilled shell portion of the roll formed of hard alloy metal in which the gradual carbon or graphite segregation has been heretofore described. Various rolls constructed in accordance with my invention have been cut in two and samples of the metal taken to accurately determine the exact composition of the metal at various points in the roll. The following table is illustrative of the metal compositions at a plurality of points in a typical roll made with metals of the compositions above described with the points being marked by circles identified by the letters  
 55 A to G in Fig. 4:

*Composition of metal throughout roll*

| Position        | A    | B    | C    | D    | E    | F    | G    |
|-----------------|------|------|------|------|------|------|------|
| Carbon.....     | 2.84 | 3.43 | 3.50 | 3.32 | 3.38 | 3.38 | 3.37 |
| Silicon.....    | .28  | .91  | .86  | .93  | .94  | .93  | .90  |
| Sulfur.....     | .076 | .108 | .100 | .104 | .104 | .106 | .101 |
| Molybdenum..... | .30  |      |      |      |      |      |      |
| Manganese.....  | .14  | .335 | .335 | .335 | .315 | .32  | .335 |
| Chromium.....   | .41  | .17  | .19  | .19  | .21  | .21  | .19  |
| Phosphorus..... | .38  | .33  | .36  | .34  | .37  | .35  | .35  |
| Nickel.....     | 4.05 | .73  | .73  | .73  | .72  | .73  | .71  |

It will be seen from the table that some mixing of the molten hard alloy and the softer core metal has taken place as shown, for example, by

the presence of a small amount of nickel in the core, but the segregation and identity of the different metals is generally very well preserved. Actually instead of strictly a displacement of the molten hard metal alloy by the softer metal there is a combined action of displacement and intermingling. Ordinarily the intermingling is reduced by increasing the amount of softer metal poured and increased by reducing the amount of softer metal poured. In all events the advantages and objects of the invention are achieved while insuring a very positive bond between the core and shell. 5

It should be understood that various metals other than those specifically described above can be employed in the manufacture of a roll in accordance with my invention. Primarily, however, the invention teaches the use of a hard high alloy metal for forming the chilled surface of a roll with a softer but tougher and more machinable metal being used as a core and to form the necks and wabbler portions of the roll. 10 20

While in accordance with the patent statutes one form of my invention and one manner of practicing my invention have been illustrated and described in detail, it should be appreciated that the invention is not limited thereto or thereby but is defined in the appended claims.

I claim:

1. That method of casting a composite metal roll with reduced neck portions which comprises bottom-pouring the central portion and lower neck with a hard high alloy metal, allowing the metal to stand until its outer cylindrical portion solidifies, bottom-pouring the roll with a softer metal to displace out of the mold at least part of the centrally positioned molten alloy metal but to leave the chilled alloy metal, removing the displaced metal from the mold just above the central portion of the roll, and completing the casting of the roll by top-pouring the upper neck with the softer metal. 30 35 40

2. In the manufacture of a necked metal roll for strip mills and the like, those steps which comprise bottom-pouring with a tangential flow a roll mold having its axis substantially vertical, said bottom-pouring being continued until the mold is filled to a point just above the central roll portion, surface chilling the central portion of the roll to form a cylindrical shell of solidified metal, continuing the bottom-pouring but with a different metal to force at least part of the still molten portion of the first metal out of the lower neck and central roll portion, withdrawing from the mold the first metal as displaced from the central portion of the roll, and top-pouring the upper neck of the roll with the different metal. 45 50 55

3. In the manufacture of a necked metal roll for strip mills and the like, those steps which comprise bottom-pouring a roll mold having its axis substantially vertical, said bottom-pouring being continued until the mold is filled to a point above the central roll portion, chilling the central portion of the roll to form a cylindrical shell of solidified metal, continuing the bottom-pouring but with a different metal to force the still molten portion of the first metal at least out of the lower neck, withdrawing the first metal as displaced from the mold at a point immediately above the central portion of the roll, closing the withdrawing port, and top-pouring the upper neck of the roll with the different metal. 60 65 70

4. That method of casting a roll with a large central portion and reduced bearing necks which comprises casting the central portion of the roll 75

against a chill and while the metal radially inside of the chilled surface metal is still molten displacing the molten metal by a swirling flow of a core forming molten metal, removing the displaced metal directly as it leaves the central portion of the roll, and completing the casting of the roll by pouring the remainder of the roll with the core forming metal with the pouring being in substantially the opposite direction to the displaced metal flow.

5. That method of casting a roll with a large central portion and reduced bearing necks which comprises casting the central portion of the roll against a chill and while the metal radially inside of the chilled surface metal is still molten displacing the molten metal by a swirling flow of a core forming molten metal, removing the displaced metal directly as it leaves the central portion of the roll, and completing the casting of

10 the roll.

15 6. That method of casting a roll with a large central portion and reduced bearing necks which comprises casting the central portion of the roll,

chilling the roll surface, and while the metal radially inside of the chilled surface metal is still molten displacing the molten metal by a core forming molten metal, and removing the displaced metal from the mold directly as it leaves the central portion of the roll.

7. That method of casting a composite metal roll having a working portion and neck portions which comprises bottom-pouring the working portion and lower neck portion with one metal, 10 allowing the metal to stand until the outer part of the working portion of the roll solidifies, bottom-pouring the roll with a second metal to displace at least part of the molten first metal but to leave the solidified outer part of the first metal, removing the displaced first metal from the mold just above the working portion of the roll, and completing the casting of the roll by pouring with the second metal the upper neck portion at a point above the working portion of 15 the roll.

20 HARRY E. WALTERS.